

# UNITED STATES PATENT OFFICE.

ROBERT C. TOTTEN, OF PITTSBURG, PENNSYLVANIA.

## CAST METAL.

947,263.

Specification of Letters Patent. Patented Jan. 25, 1910.

No Drawing.

Application filed May 19, 1909. Serial No. 497,107.

To all whom it may concern:

Be it known that I, ROBERT C. TOTTEN, a resident of Pittsburgh, in the county of Allegheny and State of Pennsylvania, have invented a new and useful Improvement in Cast Metal; and I do hereby declare the following to be a full, clear, and exact description thereof.

My invention relates to a new composition of cast metal, its object being to provide a casting metal for the production of chill castings, such as car wheels, chill rolls and the like and to produce castings of great strength of body and hard wearing surface without the employment of chilling cast iron or by the employment of a relatively small proportion thereof.

It consists, generally stated, in a composition of casting metal containing cast iron, nickel and a chromium compound containing combined iron and carbon such as ferro chrome; the nickel increasing the strength and controlling the depth of chill in the cast iron while the chromium compound increases the hardness of the surface formed and provides combined carbon and iron which furnishes the necessary combined carbon to produce the chill, or reduces the proportion of chilling cast iron necessary to be used in the casting metal, the result being a casting metal having great strength of body and high wearing properties.

In the employment of the invention I use principally iron smelted by the use of coke or coal and which contains a large proportion of graphitic carbon and only a very small proportion, sometimes only a trace, of combined carbon. I also employ nickel and ferro chrome or like chromium compound containing iron, the ferro chrome usually containing a large proportion of combined carbon, ranging as high as 10 to 12 per cent. I also employ nickel in suitable proportion, it being preferred that the chromium present shall be about 30/100 (.30) to about 70/100 (.70) per cent. of nickel in the mixture. I may also employ a chilling cast iron either in pig metal form or in the form of old car wheels and where the same is employed the proportion of nickel employed varies according to the depth of chill to be produced and the proportion of old car wheels in the casting metal and the increased strength to be given to the casting, as the nickel increases

the tensile strength of the metal and also acts to decrease the depth of chill and where such old car wheels are employed, which are liable to form a deep chill, by increasing the proportion of nickel, the depth of the chill can be regulated.

The ferro chrome provides a large proportion of combined carbon, and in proportion as it is employed a greater quantity of ordinary coke or coal iron may be employed, the chrome furnishing the combined carbon to give chilling qualities to the metal. For some purposes I may also employ steel to add to the strength of the casting metal, the proportion of steel also depending upon the amount of chilling cast iron used in the casting metal. The several metals can be varied as desired according to the character of the metal to be produced, the desired strength in the casting and the depth of chill required. The several metals may be combined in any desired way, the coke or coal iron, the chilling cast iron and steel, if the same are used, being melted in the cupola or like furnace with the ferro chrome and nickel, or the ferro chrome and nickel may be formed as an alloy, a suitable proportion of cast iron being used with the same, and the resultant alloy be melted in the furnace with the other metals or be introduced in the molten metal before the casting is formed, or the ferro chrome and nickel may be introduced separately. The casting metal so formed is of very high tensile strength and has a very hard wearing surface produced by both the combined carbon in the metal and the chromium present therein and these results are obtained either without the presence of any chilling cast iron or with a relatively small proportion thereof.

What I claim is:

1. A new composition of chilling cast metal containing cast iron, nickel and a chromium compound containing combined iron and carbon.

2. A new composition of chilling cast metal containing coke or coal iron, nickel and a chromium compound containing combined iron and carbon.

3. A new composition of chilling cast metal containing chilling cast iron, coke or coal iron, nickel and a chromium compound containing combined iron and carbon.

4. A new composition of chilling cast

metal containing chilling cast iron, coke or coal iron, steel, nickel and chromium compound containing combined iron and carbon.

5. A new composition of casting metal containing coke or coal iron, steel, nickel and a chromium compound containing combined iron and carbon.

6. A new composition of chilling cast

metal containing coke or coal iron, nickel and ferro chrome.

In testimony whereof, I the said ROBERT C. TOTTEN, have hereunto set my hand.

ROBERT C. TOTTEN.

Witnesses:

G. H. RANKIN,  
JOHN F. WILL